

# UNITED STATES PATENT OFFICE.

JOSEF LEIDL, OF NUEREMBERG, GERMANY.

## PROCESS OF MAKING TRACING, REPRINTING, AND TRANSFER PAPER.

SPECIFICATION forming part of Letters Patent No. 355,022, dated December 28, 1886.

Application filed August 10, 1886. Serial No. 210,566. (No specimens.)

*To all whom it may concern:*

Be it known that I, JOSEF LEIDL, a resident of Nuremberg, Germany, have invented an Improved Process of Making Tracing, Re- 5 printing, and Transfer Paper, of which the following is a complete specification.

Lithographers' transfer-paper as heretofore made is objectionable, because liable to be drawn out of shape. The object of my invention is to render such paper absolutely inelastic, so that it cannot be drawn out of shape, and to make it capable of being washed, at the same time leaving it transparent, fine, and pliable. On this paper the finest drawings and sketches can be executed, to be transferred to lithographic stone, even if the drawing should be several days old. The drawing can also be partly or wholly washed off and renewed. No manipulation to which the paper 20 will be exposed will draw it out of shape. It will always retain its original form. The paper is applicable to all uses to which such transparent paper can be put.

I produce the paper as follows: I first cover 25 the surface of a lithographic stone, which has the size of the paper to be treated, with boiled linseed - oil, which I apply with a roller. I place the paper upon the stone so prepared and put upon its top a light sheet of zinc or 30 other sheet and draw the stone carrying the paper and its covering through a lithographic press. This causes the linseed - oil to thoroughly permeate the paper. The paper is now taken from the stone, turned around, and 35 treated on its other face the same as described, after which it is taken off and hung up to dry. When nearly dry, which is after about twenty-four hours, the paper is once more subjected to the same treatment. The paper having 40 been thus prepared and allowed to become about half dry, is next covered with a mixture composed of about two parts of siccative coach- varnish and one part of pure odorless turpen- tine. For this purpose the paper is placed 45 upon a smooth plate of glass or the like, and is covered on both sides with said mixture

with the aid of a soft brush. It is then hung up to dry, which requires about twenty-four hours. The dry paper is then placed upon a sheet of zinc, and with a soft sponge washed 50 with soap and water, then rinsed with clean water, again well dried, and on a clean lithographic stone drawn once more through the lithographic press. Finally, it is drawn through and finished in an ordinary glazing-machine. 55 The paper thus prepared can be readily washed and cannot be drawn out of shape, as has already been stated. When to be drawn upon, it is immediately before use placed between two sheets of clean and smooth paper 60 and slowly rubbed with a palette - knife or folding - bone.

To use it as a transfer paper, it is manipulated as follows: From the original, which may be an engraved or lithographed stone, is made 65 a strong dry transfer on said paper, and the latter then in a dry condition is pressed on another stone. The last - mentioned stone, which must be clean and dry, is now rubbed with fibrous gypsum and lightly etched, and 70 then the printing color is rolled into it, so that the complete drawing becomes pereceivable. It is then etched again. Finally, the drawing is washed from the stone, the final color for printing rubbed in, and the printing pro- 75 ceeded with.

I claim—

The process herein described of preparing tracing, reprinting, and transfer paper, which consists in first coating said paper with boiled 80 linseed - oil, then pressing the same, and in finally covering it on both sides before the oil is quite dry with a mixture of siccative coach- varnish and turpentine, substantially as herein shown and described.

The foregoing specification of my improvement in tracing, reprinting, and transfer paper signed by me this 20th day of July, 1886.

JOSEF LEIDL.

Witnesses:

ANDR. STICK,  
FRIEDR. SCHATZ.